

F. HASSELMANN.  
WOOD PRESERVING SOLUTION.  
APPLICATION FILED MAY 11, 1909.

971,194.

Patented Sept. 27, 1910.



WITNESSES:

G. V. Rasmussen  
Emerson Young

INVENTOR  
FRITZ HASSELMANN

BY  
Borsig & Knabe  
ATTORNEYS

# UNITED STATES PATENT OFFICE.

FRITZ HASSELMANN, OF MUNICH, GERMANY.

## WOOD-PRESERVING SOLUTION.

971,194.

Specification of Letters Patent. Patented Sept. 27, 1910.

Application filed May 11, 1909. Serial No. 495,212.

To all whom it may concern:

Be it known that I, FRITZ HASSELMANN, a subject of the Emperor of Germany, and resident of Munich, Bavaria, Germany, have 5 invented a certain new and useful Improvement in the Art of Preserving Wood, of which the following is a specification.

My invention relates to the preserving of wood and has for its object to provide an 10 improved material with which to impregnate wood, whether fresh or seasoned. The application of my material to wood to be preserved should preferably be made according to a method which I have invented 15 and which I describe herein.

Impregnating wood with solutions of iron salts and alum in the presence of kainite, for the purpose of preserving the same, is well known, having been patented to me in the 20 United States June 6, 1899, and numbered 626,538. Without the kainite such solutions have been found incapable of penetrating the wood to a depth sufficient to bring about its artificial petrification and even with the 25 addition of kainite, which mineral often contains a sulfate of potassium and magnesium as well as a certain percentage of magnesium chlorid, satisfactory results are not to be attained. This failure is chiefly due 30 to the formation of iron-sulfur salts resulting from the dilution of the solution which occurs in boiling processes owing to the condensation of steam; or which takes place in cases where the solution is very weak. 35 These iron sulfur salts rot the wood, which, therefore, instead of being preserved, is only destroyed the more quickly. Often free sulfuric acid is formed as well as iron sulfur salts and this acid attacks the wood fibers 40 and the vessel containing the solution so that neutralization by an addition of suitable reagents becomes necessary.

According to my invention and the method herein set forth the defects just mentioned are avoided and a method and material is provided by means of which wood, whether fresh or well seasoned, is very perfectly preserved. The invention applies particularly to resinous woods, as, for example, fir.

A special advantage of my invention is that it enables the wood to be given a certain degree of hardness without sacrificing anything with respect to its preservation 55 and without affecting its color.

Referring to the drawings Figure 1 is a

front elevation and Fig. 2 a transverse section illustrating an arrangement of apparatus by means of which my invention may be carried out.

The wood *a* which is to be treated, is arranged in alternate layers in the usual manner upon a truck *b* arranged to run upon suitable rails *c* laid in a boiler *d*. This boiler may be heated by a fire maintained in 65 fire box *e*. If the wood to be treated is fresh, or only partly seasoned, it may be run into the boiler without previous preparation other than taking off the bark; but if the wood is old or has been used for any purpose, it is always best to expose fresh surfaces by planing or other equivalent method, since in surfaces which have been exposed for any length of time the pores of the wood are apt to be clogged and closed so as to absorb with difficulty, if at all. The solution *f* with which the boiler is partially filled, and with which the wood is to be impregnated, should consist preferably of about 1½% of iron chlorid ( $Fe_2Cl_6$ ), about 2% of ammonium alum, and from 1½% to 2% of magnesium chlorid, the solution being thus employed at a concentration of about 5%. A sufficient amount of solution should be used to completely cover the wood and preferably 75 to have a depth over the top of the wood equal to about  $\frac{1}{3}$  the diameter of the boiler. The heating should be regulated so as to raise the solution to a temperature of from 80° to 100° C. At this temperature the albumen 80 contained in the wood will coagulate and the rosin and other sap constituents will be chemically transformed; fungi and other living organisms will of course be absolutely 85 destroyed. The solution which is absorbed 90 tends to preserve and harden the cell walls and cause the cell structure as a whole to become of greater density and closer texture; briefly a species of petrification takes place. The wood so prepared will take a very 100 durable and high polish similar to that given to agate or other hard minerals; this makes wood so treated desirable for furniture and in the arts generally since veneer becomes superfluous. As the solution is absorbed by 105 the wood in the course of the treatment, its level gradually sinks and provision is therefore made for supplying an additional quantity of solution from time to time to maintain said level constant. This supply 110 is controlled automatically by means of a float arrangement comprising a float *g* con-

nected through a chain and lever to a valve *h* closing an inlet pipe *i* leading from a suitable reservoir (not shown) which contains the reserve supply of solution. As the level sinks, the valve is opened by the falling float, and remains open until the rise of level resulting from the incoming supply again closes the valve.

In order to secure the best results the solution should be continuously agitated during the impregnating process so as to keep it homogeneous. If this is not done the heavier metal salts will deposit more densely at the bottom than at the top and color effects in particular will be uneven. This agitation is a necessary incident of heating the boiler by direct firing, as shown in the drawings, since convection currents are of course established which keep the liquid in circulation. In case any mode of heating is used which does not establish convection currents, the system of coiled perforated pipes *j* may be used; into these pipes dry air may be forced and this air, after rising through the solution, will leave the boiler through the safety valve *h* at the top. If hot air is used the pipes *j* will serve both to heat and to stir the solution. Or, a fan arrangement *k* may be used to agitate the impregnating fluid.

The wood should be allowed to remain in the solution at the temperature previously mentioned for from two to five hours, the exact time depending upon the quality, dimensions and intended use of the wood which is being treated. At the end of this time the boiler is allowed to cool slowly and during this cooling a further absorption of solution will take place. Proceeding in this way I prevent surface cracks such as might later occur and particularly cracking of the wood near its surfaces. Cooling having taken place, the wood should be withdrawn from the boiler, drained and then carefully dried, either by stacking it in the open air, or in special and suitable drying chambers. During this drying operation a chemical change takes place and the solution is permanently fixed so that it cannot be washed out even if immersed in salt water. The color will depend upon the relative proportions of the constituents used to make up the solution. Silver grays, yellows or browns, as also any shades lying between these colors are readily obtained in this way.

It will, of course, be understood that substances capable of conferring special desired properties upon the wood may often be added to the solution with desirable results.

For example, I may add schoenit for the purpose of keeping out ants, teredos and other insects. This is particularly important when wood is to be used in the tropics. Schoenit is also useful in that it gives in-

creased hardness and improved fire-resisting qualities to wood; it can be used for this purpose in place of ammonium alum, thus proving convenient in places where the latter, for any reason, cannot be obtained. By adding potassium chlorid eminent fire proof properties are bestowed upon the wood; potassium chlorid also has an effect upon color tints, especially when used with firs and pines and by its addition causes said tints to be produced of a dark gray, dark green and other dark shades. The exact tint produced depends upon the characteristics of the wood itself. The same solution may be repeatedly used; any precipitated residue should, however, be removed after each treatment before additional or supplemental solution is introduced and after 7 to 10, treatments the entire body of solution in the boiler should be renewed or purified preferably chemically.

The improvements herein set forth are valuable in connection with wood of all kinds, but of special value in connection with wood rich in rosin, as for example the fir, pine and similar woods. I find that fir particularly, when treated according to my method, acquires in many respects the qualities of oak. This is of manifest commercial importance owing to the much larger supply of fir than oak.

In the specification preceding I have given certain preferred proportions, which I have found to be the most satisfactory in practice, for the solution in carrying out this my invention; but I have also found that these proportions may be varied somewhat without losing too largely the valuable properties desired, and I do not confine myself therefore necessarily to the exact proportions which have been set forth in the specification as preferable, but claim as my invention:

1. A solution for preserving wood, said solution containing iron chlorid, ammonium alum and magnesium chlorid in substantially the proportions specified.

2. A solution for preserving wood, said solution containing approximately 1.5% of iron chlorid, 2% of ammonium alum and from 1.5 to 2% of magnesium chlorid.

3. A solution for preserving wood, said solution being composed of a solution in which iron chlorid, ammonium alum, and magnesium chlorid have a concentration of approximately 5% to 5.5%.

In testimony whereof I have hereunto set my hand in the presence of two subscribing witnesses.

FRITZ HASSELMANN.

Witnesses:

LOUIS D. MUELLER,  
MATHILDE K. HELD.